

## UNITED STATES PATENT OFFICE

1,942,541

## METHOD OF MAKING SEAMLESS TUBES

Jerry J. Dunn, Ellwood City, and Peter C. Patterson, McKeesport, Pa., assignors to National Tube Company, a corporation of New Jersey

No Drawing. Application April 19, 1930  
Serial No. 445,819

3 Claims. (Cl. 80—62)

This invention relates to the manufacture of seamless tubes and more particularly to a method of producing large diameter, thin-walled tubes of commercial lengths.

5 Heretofore it has been the general commercial practice in manufacturing seamless tubes to heat a solid blank up to the desired temperature, then pierce the blank to form a tube having a diameter somewhat larger than the finished tube and a  
10 wall thickness of about one hundred and forty per cent. greater than the wall of the finished tube. This roughly formed tubing is then rolled in the plug rolling mill to reduce the wall thickness and to reduce the diameter to somewhat less than the finished diameter required.

The reduced tube is then passed directly and without reheating through cross-rolling machines for the purpose of smoothing the surface and equalizing the wall thickness without any  
20 material change in the wall thickness. However, during this last operation, the diameter of the tube is slightly enlarged beyond the diameter of the finished tube. The tube resulting from this last operation is then passed through sizing  
25 rolls to reduce it to final finished diameter.

The well known and commercial method described above is practical and successful on tubes up to approximately four inches in diameter, having the commercial range of wall thickness.

30 In such method, involving only a single piercing operation, the pierced billet is generally taken directly to the plug rolling mill. The temperature changes in the piercing operation are comparatively slight and not sufficient to affect the  
35 plug rolling operation.

For tubes beyond about four inches in diameter, a single piercing process involves a very large amount of work and a rapid deformation of the metal, which tend to injure the material or to  
40 destroy its appearance even when its strength is not injured. On the other hand, the use of a double or other multiple piercing operation, while free from the bad features of the single operation, will introduce a variation in temperature, causing difficulties in the subsequent rolling operations, namely—a tendency to tear the metal and a decrease in the yield of salable product.

We have discovered that by a comparatively short reheating operation the doubly pierced  
50 product can be rolled without producing these defects. The reheating serves to off-set two incidents to the double piercing. The double piercing operation increases the time interval between the moment when the metal leaves the initial heating furnace and the moment when

it enters the rolling mill, and thus involves a considerable cooling of the work. But the original temperature cannot be varied except within a narrow range, not sufficient for our purpose because to do so interferes with the success of the 60 piercing operation. The difficulty, due to cooling by double piercing, is particularly apparent when the ratio of wall thickness to outside diameter in the finished tube is within less than about three per cent.; that is, what may be called "thin-walled" tubes. Not only is there a 65 material lowering of the temperature of the tube as a whole but there is also a considerable variation in its temperature from end to end, due to the nature of the second piercing operation, bringing the wall thickness to about one-half or one-third of that produced in the first piercing 70 operation.

We have found, however, that with an initial temperature suitable for piercing and with a 75 short reheating after piercing, the difficulties referred to can be obviated and tubes of large size and great length and comparatively thin walls can be produced with an increased percentage of salable yield and an improved quality of the product.

The tube after the last piercing operation needs to be left in a reheating furnace only a few minutes, one or two minutes generally, in order to make it suitable for successful rolling and also to unify the temperature from end to end within practical limits.

The most important effect of this reheating is the capability of producing the tubes in comparatively great lengths by rolling them at a temperature which is approximately uniform from end to end. This unifying of the temperature is due largely to the mere holding of the tube between the last piercing and the first rolling operation, since there is always a tendency for the heat to distribute itself fairly rapidly throughout the length of the highly conductive steel; and the value of the reheating operation is largely in preventing loss of heat during such unifying period while the total heat of the tube is being averaged throughout its length.

In view of our discoveries we therefore have developed a practical and successful method of producing commercial, thin-walled seamless tubes having a greater diameter than about four inches which consists in heating a round solid blank or billet to the proper piercing temperature, piercing the heated billet to form a rough tube having a wall thickness of from approximately 340 to 440 per cent. greater than the 105 110

wall thickness of the finished tube, then again piercing the once pierced tube without reheating to increase its diameter and reduce its wall thickness to approximately 140 per cent. greater than 5 the wall thickness of the finished tube.

Due to this double piercing step, the tube blank is too cool and its temperature too uneven to permit successful plug rolling; therefore, we next pass the tube into a temperature equalizing furnace where the tube is brought to an equal temperature throughout its length suitable for 10 the further finishing operation. The tube is generally retained in the reheating furnace from one to two minutes.

15 After the temperature of the tube has been equalized and brought to the proper plug rolling temperature it is plug rolled, cross-rolled and sized in the usual manner without further heating and results in the production of a large diameter (a diameter of more than four inches) thin-walled tube of commercial length, a thin-walled tube being that in which the ratio of wall thickness to outside diameter approximates one and one-quarter to three per cent.

20 While we have described one specific series of steps for carrying out our invention, it will be understood that we do not wish to be limited thereto, since various modifications may be practiced without departing from the scope thereof, 25 as defined in the appended claims.

We claim—

1. The method of making thin walled seamless tubes of greater than five and one-half inches in diameter and of standard commercial lengths and 30 having a ratio of wall thickness to outside diameter less than about three per cent. which consists in heating a round solid blank or billet to the proper piercing temperature, piercing said heated billet to form a rough tube having a wall 35 thickness of from approximately 340 to 440 per cent. greater than the wall thickness of the finished tube, then again piercing said once pierced tube without reheating to increase its diameter and reduce its wall thickness to approximately 40 140 per cent. greater than the wall thickness of the finished tube, then carrying the twice pierced tube in a furnace for a brief period, of the order of one or two minutes, immediately after the last 45 piercing operation to produce a uniform temper-

50

ature from end to end of said pierced tube, then removing said uniformly heated tube and plug rolling, cross rolling and sizing said tube to finished size.

2. The method of making thin walled seamless tubes of greater than five and one-half inches in diameter and of standard commercial lengths and having a ratio of wall thickness to outside diameter less than about three per cent. which 55 consists in heating a round solid blank or billet to the proper piercing temperature, piercing said heated billet to form a rough tube having a wall thickness of several times the wall thickness of the finished tube, then again piercing said once pierced tube without reheating to increase its diameter and reduce its wall thickness materially, then carrying the twice pierced tube in a furnace for a brief period, of the order of one or two minutes, immediately after the last piercing 60 operation to produce a uniform temperature from end to end of said pierced tube, then removing said uniformly heated tube and plug rolling, cross rolling, 65 cross rolling and sizing said tube to finished size.

3. The method of making thin-walled seamless tubes of greater than five and one-half inches in 70 diameter and of standard commercial lengths and having a ratio of wall thickness to outside diameter less than about 3 per cent. which 75 consists in heating a round solid blank or billet to the proper piercing temperature, piercing said heated billet to increase its length and diameter and form a rough tube having a wall thickness of several times the wall thickness of the finished tube and less than 450 per cent. greater than the wall thickness of the finished tube, then again 80 piercing said once pierced tube without reheating to increase its length and diameter and reduce its wall thickness to less than 150 per cent. greater than the thickness of the finished tube, then carrying the twice pierced tube in a furnace for 85 a brief period, of the order of one or two minutes, immediately after the last piercing operation to produce a uniform temperature from end to end of said pierced tube, then removing said uniformly heated tube and plug rolling, cross-rolling, 90 cross rolling and sizing said tube to finished size.

JERRY J. DUNN.  
PETER C. PATTERSON.

125

55

130

60

135

65

140

70

145

75

150